

Patented Nov. 14, 1922.

## UNITED STATES PATENT OFFICE.

WILLIAM RAUTENSTRAUCH, OF TRIER, GERMANY.

## PROCESS FOR UNHAIRING SKINS AND HIDES.

No Drawing.

Application filed August 21, 1920. Serial No. 405,188.

(GRANTED UNDER THE PROVISIONS OF THE ACT OF MARCH 3, 1921, 41 STAT. L., 1313.)

To all whom it may concern:

Be it known that I, WILLIAM RAUTENSTRAUCH, merchant, residing at Trier, Germany, have invented certain new and useful Improvements in Processes for Unhairing Skins and Hides (for which I filed an application for patent in Germany on May 9, 1919), of which the following is a specification.

10 The tanning of animal hides being accompanied by the absorption of tanning matter, either by mechanical adherence or chemical combination, it would be expected that a considerable increase of weight due to the tanning process and exceeding the weight of the unhaired dry skin by the amount of absorbed tan would occur. Nevertheless by the methods usually employed a corresponding increase of weight is never obtained and this can only be explained by a loss in dermal matter compensating more or less for the weight of the tanning substance fixed by the skin.

15 The loss of dermal substance occurs during the preparation of hides and skins for the tanning process and particularly during the unhauling process. This is mostly done by the sweating process or by treating the hides with a lime bath or sulphide of sodium.

20 The sweating of hides provokes a slackening of the roots of the bristles and hair by putrefaction which also attacks and destroys the albuminoids within the skin. This results in a double loss in that the albuminous substances, as well as the tan which would have been fixed to them, are lost. Solutions of lime dissolve albumens and extract the so-called intercellular substance from the hides. The dissolved substances very soon become

25 putrid and also contaminate the hides themselves, so that the lime bath must be thrown away and renewed from time to time.

Sulphide of sodium destroys bristles and hair and damages the hides themselves.

30 Careful investigations have proved that a depilatory bath extracts the albumens dissolved in the skin only up to a point where a certain balance between the solution of albumen in the bath and that in the skin is attained. Therefore the depilatory bath should, if possible, be enriched with dermal substance and at the same time the latter must be prevented from putrefying. If pos-

sible such a depilatory should be chosen as will prevent putrefaction. 55

A chemical fulfilling these requirements is barium hydroxide or strontium hydroxide. Where a lime bath which has not a sufficient disinfecting power is used, a disinfectant suitable for that purpose, for example, creosote, should be added. It is not possible to say whether the use of such a lime bath has any later deleterious effect. A barium hydroxide bath enriched with dermal substance has been tried and gives excellent results. 60

Careful observations on practical work in tanyards made during several years proved the fact that, in a depilatory barium bath enriched up to a certain point with dermal substance protected from becoming putrid, the hides do not lose any dermal substance. 70

It has even been observed recently that so-called empty hides absorbed albuminous substance from a bath containing a large amount of the latter, thus improving their quality. 75

The enrichment of the bath with dermal matter may be cheaply effected by the addition of parings of hides, decay of skins, ears, muzzles, etc., in the freshly prepared depilatory. 80

A barium hydroxide or strontium hydroxide depilatory after having been used for unhauling hides for a sufficient time to be saturated with dermal matter may also be used. Up to the present time those experimenting with barium hydroxide as depilatory did not wait till the point just mentioned was attained, but emptied and renewed the bath as usual from time to time. This explains the unsatisfactory results obtained hitherto with barium hydroxide as a depilatory. 85

It has already been suggested to add albumen or albuminous matter to lime or caustic alkali as depilatory, but a lime depilatory containing albumen very soon becomes putrid and caustic alkali very soon decomposes albumen, hence it is not possible by these methods to realize the purpose of enriching a depilatory for a certain period with albuminous substance. 90

The hairs, bristles and paring of the hides after treatment according to my process are 105 of the very best quality.

The process can be used for any sort of skin, hide or leather.

Special apparatus for carrying out the process are not required.

5 Claim.

A process for unhauling skins or hides, which process consists in dissolving barium hydroxide in water, adding to the solution hide substance until no more will dissolve

therein, soaking the skin or hide to be treated 10 in the liquid and finally removing the hair from the skin or hide.

In testimony whereof I affix my signature in presence of two witnesses.

WILLIAM RAUTENSTRAUCH.

Witnesses:

CHARLES DUMONT,  
H. SCHAEFER.